# EUROPEAN PATENT SPECIFICATION

(11) **EP 0 708 852 B1**
(45) Date of publication and mention of the grant of the patent: **18.03.1998**
(21) Application number: 94920307.9
(22) Date of filing: 29.06.1994
(51) Int. Cl.: D04H 1/64, D04H 1/42

(54) **NEW FIBERFILL BATTINGS**
NEUES FASERFÜLLMATERIAL FÜR MATTE
NOUVELLES NAPPES DE FIBRES DE REMBOURRAGE

(30) Priority: 01.07.1993 US 84936
(43) Date of publication of application: 01.05.1996
(73) Proprietor: E.I. DU PONT DE NEMOURS AND COMPANY, Wilmington Delaware 19898 (US)
(72) Inventor: FRANKOSKY, Michael, Stephen, Hockessin, DE 19707 (US); KWOK, Wo, Kong, Hockessin, DE 19707 (US)
(74) Representative: Jones, Alan John
(86) International application number: US9407076
(87) International publication number: WO9501475

(56) References cited:
- EP-A- 0 265 221
- EP-A- 0 314 433
- EP-A- 0 437 268
- WO-A-80/01031
- WO-A-93/11292

## Description

This invention is concerned with improvements in and relating to bonded polyester fiberfill batts, sometimes referred to as battings, especially such improved batts with desirable aesthetic and serviceable qualities, and to articles incorporating such improved batts.

In parent U.S. Patent No. 5,225,242 and WO 93/11292, the disclosures of which are incorporated herein by reference, we provided a process for preparing a bonded batt, comprising forming a blend of polyester fiberfill, in amount by weight about 70 to about 96%, intimately mixed with a binder fiber, preferably a bicomponent binder fiber, having binder material of melting point lower than the softening point of the polyester fiberfill, in amount by weight about 4 to about 30%, preparing a continuous batt from said blend, said batt having an upper face and a lower face, advancing said batt through one or more spray zones, whereby both faces of the batt are sprayed with resin, in total amount about 10 to about 30% of the weight of the sprayed batt, including the resin, said resin being selected to provide, after curing, a cured resin having a glass transition temperature (Tg) of about 0 degrees Celsius or less, heating the sprayed batt in an oven to cure the resin and soften the binder material, followed by hot-rolling the heated batt to achieve intimate contact between the resin and the fibers in the faces of the batt, and cooling the rolled batt, such hot-rolling being preferably effected by use of heated rolls in a calender or S-wrap configuration, and bonded batts of improved aesthetics and performance such as were made by such a process. The weight of the fibers in the batt (i.e., of the blend of polyester fiberfill and of binder fiber) is referred to as the "basis weight" of the batt, i.e., before the sealing resin is sprayed on.

We have, however, according to the present invention, found that, surprisingly, hot rolling need not necessarily be performed to impart adequate sealing, provided low denier fiberfill (referred to variously as subdenier or microfibers) is used to help with sealing at least in one or both face(s) of the batt. Thus, there is now provided a bonded batt, with upper and lower faces, said batt comprising polyester fiberfill of denier per filament greater than 0.2 and not more than 1, in amount about 75 to about 96%, and bonded throughout with lower melting binder material, complementally in amount about 4 to 25%, said amounts being calculated on the basis weight of the batt, said batt having a wash durability (WD, as defined) of at least 4, and a bending stiffness (B, as defined) of about 40 cN/cm² or less, wherein at least one of said faces is sealed with a resin having a glass transition temperature (Tg) of about 0 deg Celsius or less, in amount about 0.02 to about 0.35 oz/yd² (0.7 to 12 g/m²), preferably about 0.1 to about 0.25 oz/yd² (3.4 to 8.5 g/m²), calculated with regard to said face of the batt, whereby the sealing rating (SR, as defined) of said face is at least 4, said bonded batt having been prepared without the use of hot rolling. Preferably each of said faces is so sealed.

Both metric units, such as dtex, and denier are used herein, 1 dtex being the same as 0.9 denier per filament (dpf).

Thus, the present invention provides fiberfill batts, such as are needed for use in premium apparel, by first preparing a homogeneous blend of polyester fiberfill (75-96% by weight of the blend) and a suitable binder fiber (4-25% by weight of the blend). This blend is converted on a card or garnet to a web which may then be layered or cross lapped to form a batting to whose upper (and preferably serially also to whose lower) face is applied a suitable latex (e.g., a colloidal dispersion of acrylic polymers and/or copolymers in water, discussed in more detail hereinafter), e.g., by spraying. The sprayed batting is heated, e.g., conveniently by being passed through a heated oven to dry the coating(s) and to polymerize the polymeric component(s) to high molecular weight, and to activate the binder fiber. This may be conveniently done, for example, in three passes through such an oven, two to serially dry and partially cure each such coating, after it has been applied to any face, and a final pass to supplement the other(s).

When the fiberfill is greater than 0.2 and not more than 1 denier per filament, however, and when said resin applied to the batting faces has a glass transition temperature (Tg) of about 0 degrees Celsius and has been applied in amounts between about 0.02 oz/yd² (0.7g/m²) to 0.35 oz/yd² (12 g/m²), then additional treatment, as with hot rolls, is not undertaken to prevent fiber leakage, especially when dry fiberfill is used.

The resins that may be used herein are termed variously, by different manufacturers, as "soft" or "medium", or even "very soft", but are characterized by having second order glass transition temperatures (Tg) of about 0 C or less. They provide both softness and drapability to the batt when used in, e.g., apparel, while acting as barrier to fiber leakage from the batt. The final batts may have a basis weight of 1.5 to 12 oz/yd² (50 to 400 g/m²) and a thickness of 0.07 to 0.20 inch/oz/yd²(0.05 to 0.15 mm/g/m²). Thus the batts of this invention are prepared from a blend of polyester fiberfill and binder fibers, and the fibers in the face(s) are sealed by a suitably soft-type resin coating. The polyester fiberfill may all be slickened, e.g., as described herein, or may be a blend of slickened and unslickened fibers. The fiberfill may be solid, hollow, or a blend of solid and hollow fibers and is not limited to any type of fiber cross section, i.e., it may be of cruciform, trilobal, Y-shaped, dog bone, scalloped oval, and other non-circular cross sections as well as round. The fiberfill has a denier per filament (dpf) within the range of 0.2 to 10, with a dpf of about 1.65 being very useful, and constitutes about 70 to 96% by weight of the blend. As indicated, subdenier fibers give good sealing in the face(s) of the bonded batt, so are often preferred in such face(s). The individual fibers are provided with crimp by conventional means and typically exhibit from 5 to 15 crimps per inch (cpi) and have a length within the range of 3/4 to 3 inches. The binder fibers constitute from about 4 to 30% by weight of the batt and may be of the sheath/core (s/c), side/side (s/s), or monocomponent types. These may be obtained from (co)polyesters, polyolefins, polyolefin/polyester, polyamide/polyamide, e.g., and the like. Useful types of binder fibers, and their modes of functioning, are described in, e.g., "Nonwovens World", March/April, 1990, page 37. The initial dpf of suitable binder fibers in the blend is typically within the range of 2 to 15 with a dpf of 4 being commonly used. Useful binder fibers include those disclosed in the aforementioned U. S. Patents to Scott, Pamm, Frankosky, and Marcus, together with those shown in Harris et al U. S. Patent No. 4,732,809; Taniguchi et al U. S. Patent No. 4,789,592; Tomioka et al U. S. Patent No. 4,500,384; Hirose et al Japanese Patent Publication Kokai 57-210,015(1982); and others known in the art which will function within the oven temperatures disclosed herein. Preferred binder fibers include the commercially-available "Melty 4080" (Unitika Co., Japan) and the "ES" and "EA" polyolefins (Chisso Corporation, Japan).

The cured resin coatings on both faces of the batt may conveniently constitute about 10 to 30% by weight of the final bonded batt, with 12 to 25% being preferred for 1.65 dpf (1.83 dtex), where lesser amounts of resin tend to reduce wash durability and sealing rating while greater amounts tend to increase stiffness and reduce insulating efficiency. If only one face of the batt is so sealed, only half as much resin need be applied. When low fiber deniers (about 1 dpf or less) are used, less resin coating is needed to achieve fiber leakage control. Moreover, the amount of resin in the surface(s) need not depend on the basis weight of the batting, and so, for heavier battings, the total resin add-on may be as little as 3%, even for slickened fiberfill batts. For entirely dry (unslickened) fibers, less resin is needed than when slickened fiberfill is used.

As noted previously, a suitable resin for coating has a Tg of about 0 C or less. The useful resins are obtained from commercially-available acrylic and vinyl latex compositions among which are included, e.g., Rhoplex E-32 (Rohm and Haas Co.), TR-934 (Rohm and Haas Co.), X-4280J (Kanebo, Japan), these Hycar® latex compositions of B. F. Goodrich Co.: 26146, 26171, 26322, 26083, 26092, 2671, 26120, 2679, 26796, these latex products of National Starch and Chemical Corporation: NACRYLIC X 4445, NACRYLIC X 788-6007, NACRYLIC X 4483, NACRYLIC X 4460, NACRYLIC X 4260, NACRYLIC X 4425, NACRYLIC X 4465, NACRYLIC 4401, NACRYLIC X 78-3990, NACRYLIC X 78-3997, NACRYLIC X 78-3905, NACRYLIC X 4280, NACRYLIC 4441, NACRYLIC 78-6114, X-LINK 2873, X-LINK 2849, X-LINK 78-6119, X-LINK 2893, X-LINK 2833, X-LINK 78-6004, X-LINK 2813, RESYN 2375, DUR-O-SET E-230, DUR-O-SET E-669, and other commercially-available latexes which are cured to resins whose Tg values are about 0 C or less. Some of such commercially-available resins and their Tg values are listed in brochures, e.g., one by B. F. Goodrich, dated 1989, entitled HYCAR® Acrylic Latexes, and one by National Starch and Chemical Corporation, entitled Binders, Saturants, Laminants.

Preparation of the batts is generally begun by conventional opening and blending of the polyester fiberfill and binder fiber, followed by carding or garnetting to make a web. This web can be layered with other webs from a train of cards or garnets, or it can be cross lapped and combined with other webs to form an unbonded batting. This batting is then sprayed with the latex composition on one or both sides of the batting and is fed to the oven for curing of the resin and bonding of the binder fibers. The oven treatment is conducted at 150-190 C for 2 to 5 minutes, and may be conveniently done in three passes of the batt, as previously noted. The batts exhibit the basis weight and thickness ranges previously indicated.

The batts of this invention exhibit desirable levels of thermal resistance or insulation, commonly reported as CLO ratings (see Hwang U.S. Patent No. 4,514,455). Batts of this invention desirably exhibit a CLO value of at least about 0.36 CLO/oz/yd² (0.01 CLO/g/m²) and preferably 0.48 CLO/oz/yd² (0.014 CLO/g/m²) or higher.

It is to be understood that the components and processes described herein should be selected to provide the batts of this invention. Care must be taken to select combinations that do so provide. For example, the slickener on the fiber and the latex applied to the batt should be selected so as to adhere sufficiently, so that the final batt may exhibit, for example, sufficient wash durability.

### TEST PROCEDURES

CLO ratings are obtained as described in Hwang, above.

Wash durability ("WD") of the batts of this invention is evaluated by the procedures of ASTM D-4770-88. In the Examples, the panels were 24 inches x 24 inches in size. Durability ratings are reported for measurements made according to paragraph 8.6.1. Batts of the invention exhibit a rating of 3 or higher (paragraph 8.5 scale).

Fiber leakage or percolation through shell fabric is measured as a sealing rating ("SR") by the method described in LeVan U. S. Patent No. 4,869,771 (after 3 wash cycles), a sealing rating (SR) of 5 being excellent and a sealing rating (SR) of 1 being poor. The batts of this invention exhibit a sealing rating (SR) of 3 or higher (after 3 wash cycles). In Table 2 (Example 3), sealing values are additionally reported after one wash (1W) as well as after 3 washes (3W) and compared with initial values before any washing (NEW).

The softness or drapability of the batts of this invention is measured according to German Industrial Standard 53362 Cantilever (DIN 53362 Cantilever) which determines and totals the bending stiffness ("B") of the batting in machine and cross machine directions; the combined results are related to drapability and softness. Batting samples are cut to 25 cm. length and 2.5 cm. width, and are cut in both machine (MD) and cross machine (XD) directions. Each Test specimen is weighed and its weight recorded as "W". Bend length ("LU") is then determined by sliding the sample horizontally on a platform until the front of the bent sample reaches an angle of 41 degrees and 30 seconds. The following calculation is then made:${\text{B = F}}_{\text{1}} {\text{(LUö2)}}^{\text{3}}$ where
- B =: bending stiffness in cN/cm.²
- LU =: bend length in cm.
- F₁ =: 9.8 (WöL)
- W =: weight of the specimen sample in grams
- L =: sample specimen length in cm.

The batts of this invention exhibit a bending stiffness ("B" being the sum of values determined for MD and XD samples from the batt) of 80 cN/cm.² or less, a lower bending stiffness being preferred.

The invention is further illustrated in the following Examples, all parts and percentages being by weight, unless otherwise indicated, calculated with regard to the "BW" (Basis Weight, i.e., to the amount of polyester filberfill and binder fiber only, (i.e., without the added resin sprayed onto the faces to improve the sealing).

### EXAMPLE

Various batting samples were prepared and tested, with results being shown in the Table. The binder fiber each time was "Melty 4080" (4 dpf), but different fiberfill fibers were used.

Samples A, B, C and D were prepared from a commercially-available blend of polyester fibers consisting of 37.5% of slickened 1.65 dpf (finished with a silicone slickener), 37.5% of dry 1.65 dpf (without any silicone slickener), and 25% binder fiber. The blend was processed on conventional card and cross-lapper equipment similar to the equipment as described in Example 1 of U.S. Patent No. 5,225,242. The resulting battings were fed through a triple-pass oven maintained at about 165 C. The battings (except for A) were sprayed with equivalent amounts of a soft resin (glass transition temperature (Tg) equals -10 deg C) on each side such that the total resin add-on was as stated in the Table, based on "BW", the basis weight of the fiber in the batting at this stage which was about 4.5 oz/yd²(150 g/m²). One side of the batting was sprayed with resin before entering the first pass and the other side was sprayed before entering the second pass. Importantly, the entire batting was exposed to adequate time at a temperature sufficiently high to assure complete cure of the resin and set of the binder fiber (1 minute after the batt has reached 165 C has generally been sufficient). The battings were then calendered in a separate operation which served to seal the surfaces and reduce loft.

From the Sealing Values in the Table, it can be seen that, under these conditions, even with 8% resin (Sample B), the effect of calendering did not improve the sealing of the 1.65 dpf fibers batt after 1 wash cycle, and even with 15% resin (Sample C), the sealing was improved after 1 wash cycle, but still inadequate after 3 cycles. At 25% resin, under these conditions, the Sealing Rating of the surface of Sample D was satisfactory (after three wash cycles).

The battings were also tested for fiber leakage by encasing in a fabric with a yarn count of 104 X 84, and a Frazier air permeability rating of 13.2 cu ft/min at a pressure drop of 0.5 inches of water.

Samples E and F were the same as Samples A and D, respectively, except these were tested in a fabric with a yarn count of 102 x 84 and a Frazier rating of 48. Since 0.7 dpf battings were also tested in a more permeable fabric than for Samples A-D, results on Samples E and F (1.65 dpf) are included in the Table to bridge the data between Samples A-D and G-Q. Sample E, without resin, failed when new because of the openness of the fabric, but after three wash cycles had become sufficiently matted that it improved its leakage performance. Sample F's Sealing Value was 5 initially and provided a satisfactory Sealing Rating, i.e., after 3 wash cycles).

Samples G, H, I and J were prepared from a blend of about 85 pounds of dry polyester fibers (0.7 dpf, 0.78 dtex, 1.5 inch cut, 12 cpi, without any special slickening finish) and 15 pounds of binder fiber. These samples were resin-sprayed, calendered and tested as for samples E and F.

Samples K and L were prepared from a blend of about 55 pounds of similar 0.7 dpf slick fiber, finished with a silicone slickener, 27 pounds of dry (unslickened) 0.7 dpf fiber, and 18 pounds of binder fiber. These samples were not calendered, as indicated by the double asterisks in the Table, but gave good sealing ratings.

Samples M, O, P and Q were similarly prepared from the same kind of blend as K and L, but were made to higher basis weights, as shown, and also showed good sealing ratings, despite lower (less than 10%) resin add-on and despite not being calendered, because of use of low dpf fiber. N was calendered (unlike the others). A comparison of these results shows that calendering was not needed to improve the sealing rating (when the subdenier fibers were used with the soft resin).

Samples G through L were all tested for fiber leakage using the 48 Frazier fabric.

Accordingly, in the Table, samples K-M and O-Q are all according to the invention, whereas the others show comparisons, some without any resin sprayed on, some with regular denier fiberfill and whose sealing ratings are not adequate after washing, and some which were calendered.

**TABLE**

| | Frazier | BW | Fiber dpf | Resin | | | Sealing Values | |
|---|---|---|---|---|---|---|---|---|
| | | | | % | * (g/m²) | New | 1W | 3W |
| A | 13.2 | 4.5 | 1.65 | 0 | 0 (0) | 5 | 1 | 1 |
| B | 13.2 | 4.5 | 1.65 | 8 | 0.36 (12.2) | 5 | 1 | 1 |
| C | 13.2 | 4.5 | 1.65 | 15 | 0.67 (22.7) | 5 | 3 | 1 |
| D | 13.2 | 4.5 | 1.65 | 25 | 1.125 (38.1) | 5 | 5 | 5 |
| E | 48 | 4.5 | 1.65 | 0 | 0 (0) | 1 | 1 | 4 |
| F | 48 | 4.5 | 1.65 | 25 | 1.125 (38.1) | 5 | 5 | 5 |
| G | 48 | 4.5 | 0.7 | 4 | 0.18 (6.1) | 5 | 5 | 5 |
| H | 48 | 4.5 | 0.7 | 2.2 | 0.10 (3.4) | 5 | 5 | 5 |
| I | 48 | 4.5 | 0.7 | 1.6 | 0.07 (2.4) | 5 | 5 | 5 |
| J | 48 | 4.5 | 0.7 | 0 | 0 (0) | 4 | 1 | 1 |
| K** | 48 | 4.5 | 0.7 | 10 | 0.45 (15.3) | 5 | 5 | 5 |
| L** | 48 | 4.5 | 0.7 | 5 | 0.225 (7.6) | 5 | 5 | 5 |
| M** | 48 | 6.1 | 0.7 | 6 | 0.37 (12.5) | 5 | 5 | 4 |
| N | 48 | 5.1 | 0.7 | 7 | 0.36 (12.2) | 5 | 5 | 5 |
| O** | 48 | 8.0 | 0.7 | 6 | 0.48 (16.3) | 5 | 5 | 5 |
| P** | 48 | 8.1 | 0.7 | 8 | 0.65 (22.0) | 5 | 5 | 5 |
| Q** | 48 | 9.3 | 0.7 | 5 | 0.47 (15.9) | 5 | 5 | 5 |

| | | | | | | | | |
|---|---|---|---|---|---|---|---|---|
| * indicates the total amount of resin sprayed on (both surfaces of) the batt, calculated in oz/yd² and g/m² (half these amounts indicate the amounts on each face). | | | | | | | | |
| ** indicates there was no calendering after oven cure | | | | | | | | |

## Claims

1. A bonded batt with upper and lower faces, said batt comprising polyester fiberfill of denier per filament greater than 0.2 and not more than 1, in amount about 75 to about 96% and bonded throughout with lower melting binder material, complementally in amount about 4 to 25%, said amounts being calculated on the basis weight of the batt, said batt having a wash durability (WD) of at least 4, and a bending stiffness (B) of about 40 cN/cm² or less, wherein at least one of said faces is sealed with a resin having a glass transition temperature (Tg) of about 0 deg Celsius or less, in amount about 0.7 g/m² (0.02 oz/yd²) to about 12 g/m² (0.35 oz/yd²), calculated with regard to said face of the batt, whereby the sealing rating (SR) of said face is at least 4, said bonded batt having been prepared without the use of hot rolling.

2. A batt according to Claim 1, wherein the amount of resin is about 3.4 to about 8.5 g/m² (about 0.1 to about 0.25 oz/yd²).

3. A batt according to Claim 1 or 2, wherein each of said upper and lower faces is sealed with said resin in said amount and has a sealing rating of at least 4.

4. A process for preparing a bonded batt in accordance with Claim 1, Claim 2 or Claim 3, which process comprises preparing a homogeneous blend of 75-96% by weight of said polyester fiberfill and 4-25% by weight of said binder material in the form of fiber, converting the blend on a card or garnet to a web which is layered or cross lapped to form a batt, applying said resin to the upper face of said batt, and heating the batt to cure the resin and bond the binder fibers, and wherein hot rolling is not performed on the batt.

5. A process according to Claim 4 wherein the resin is sprayed onto the batt.

6. A process according to Claim 4 or Claim 5 wherein the batt is heated in three passes through a heated oven.

## Patentansprüche

1. Gebundenes Vlies mit einer Ober- und einer Unterseite, wobei das Vlies Polyester-Faserfüllstoff mit einem Denier-Wert pro Filament von mehr als 0,2 und von höchstens 1 in einer Menge von etwa 75 bis 96 % aufweist und gänzlich mit niedrigerschmelzendem Bindematerial gebunden ist, das komplementär in einer Menge von etwa 4 bis 25 % vorliegt, wobei diese Mengen in bezug auf das Flächengewicht des Vlieses errechnet wurden, wobei das Vlies eine Waschbeständigkeit (WD, wie definiert) von mindestens 4 und eine Biegesteifheit (B, wie definiert) von etwa 40 cN/cm² oder weniger aufweist, wobei mindestens eine der Seiten versiegelt ist mit einem Harz mit einer Glasumwandlungstemperatur (Tg) von etwa 0 °C oder weniger in einer Menge von etwa 0,7 g/m² (0,02 oz/yd²) bis etwa 12 g/m² (0,35 oz/yd²), berechnet in bezug auf die Seite des Vlieses, wobei der Versiegelungswert (SR) der Seite mindestens 4 beträgt, und wobei das gebundene Vlies ohne Anwendung des Warmwalzens hergestellt wird.

2. Vlies nach Anspruch 1, bei dem die Harzmenge etwa 3,4 bis etwa 8,5 g/m² (etwa 0,1 bis etwa 0,25 oz/yd²) beträgt.

3. Vlies nach Anspruch 1 oder 2, bei dem jede der Ober- und der Unterseite mit dem Harz in dieser Menge versiegelt ist und einen Versiegelungswert von mindestens 4 aufweist.

4. Verfahren zur Herstellung eines gebundenen Vlieses nach Anspruch 1, Anspruch 2 oder Anspruch 3, wobei dieses Verfahren die Herstellung einer homogenen Mischung aus 75 - 96 Gew.-% des Polyester-Faserfüllstoffs und 4 - 25 Gew.-% des Bindematerials in Faserform, das Umwandeln der Mischung auf einer Karde oder Garnettmaschine zu einem Vlies, das so geschichtet oder kreuzweise gelegt wird, daß eine Vliesmatte entsteht, das Aufbringen des Harzes auf die Oberseite des Vlieses und das Aufheizen des Vlieses zum Härten des Harzes und zum Binden der Bindefasern umfaßt, und bei dem kein Warmwalzen an dem Vlies erfolgt.

5. Verfahren nach Anspruch 4, bei dem das Harz auf das Vlies gesprüht wird.

6. Verfahren nach Anspruch 4 oder Anspruch 5, bei dem das Vlies in drei Durchläufen durch einen beheizten Ofen aufgeheizt wird.

## Revendications

1. Une nappe liée comportant une face supérieure et une face inférieure, ladite nappe comprenant des fibres de rembourrage en polyester d'un denier par filament supérieur à 0,2 et ne dépassant pas 1, en quantité d'environ 75 à environ 96% et liée dans la masse par un matériau de liaison de bas point de fusion, en quantité complémentaire d'environ 4 à 25%, lesdites quantités étant calculées par rapport au poids de base de la nappe, ladite nappe ayant une durée de vie au lavage (WD tel que défini) d'au moins 4, et une rigidité à la flexion (B, tel que défini) d'environ 40cN/cm² au moins, dans laquelle l'une au moins desdites faces est agglutinée par une résine présentant une température de transition vitreuse (Tg) égale ou inférieure à environ 0°Celsius, en quantité comprise entre environ 0,7g et 12g/m² (0,02 et 0,35oz/yd²), calculée par rapport à ladite face de la nappe, la note d'agglutination (SR) de ladite face étant au moins égal à 4, ladite nappe liée ayant été préparée sans utilisation de cylindrage à chaud.

2. Une nappe selon la revendication 1. dans laquelle la quantité de résine est comprise entre environ 3,4 et environ 8,5g/m² (environ 0,1 et environ 0,25oz/yd²).

3. Une nappe selon la revendication 1 ou 2, dans laquelle chacune desdites faces supérieure et inférieure est agglutinée par ladite résine en ladite quantité et présente à une note d'agglutination au moins égale à 4.

4. Un procédé de préparation d'une nappe liée selon la revendication 1, la revendication 2 ou la revendication 3, ledit procédé consistant à préparer un mélange homogène de 75-96% en poids de ladite fibre de rembourrage en polyester et 4-25% en poids dudit matériau de liaison sous forme de fibre, à convertir le mélange sur une cardeuse ou une peigneuse en un voile qui est déposé tel que ou déposé avec croisement, pour former une nappe, à appliquer ladite résine sur la face supérieure de ladite nappe, et à chauffer la nappe pour vulcaniser la résine et lier les fibres de liaison, et dans laquelle un cylindrage à chaud n'est pas mis en oeuvre sur la nappe.

5. Un procédé selon la revendication 4, dans lequel la résine est pulvérisée sur la nappe.

6. Un procédé selon la revendication 4 ou 5, dans lequel la nappe est chauffée en trois passes dans un un four chauffé.
